

Dec. 4, 1945.

E. J. KALIL

2,390,440

LEAD COATING

Filed May 29, 1942

2 Sheets-Sheet 1

Fig. 1.



Fig. 2.



INVENTOR.

EUGENE JOSEPH KALIL

BY

*A. Dr. Weiller*  
ATTORNEY

Dec. 4, 1945.

E. J. KALIL

2,390,440

LEAD COATING

Filed May 29, 1942

2 Sheets-Sheet 2

*Fig. 3.*



*Fig. 4.*



*Fig. 5.*



INVENTOR.  
EUGENE JOSEPH KALIL

BY

*A. D. Weller*  
ATTORNEY

Patented Dec. 4, 1945

2,390,440

# UNITED STATES PATENT OFFICE

2,390,440

## LEAD COATING

Eugene Joseph Kalil, Huntington, W. Va., assignor to The International Nickel Company, Inc., New York, N. Y., a corporation of Delaware

Application May 29, 1942, Serial No. 445,399

8 Claims. (Cl. 117—52)

The present invention relates to lead coating, and, more particularly, to a novel flux and process for coating metals and alloys with lead preparatory to a metal drawing operation.

It was known that a coating of soft metal, e. g., lead, on the surface of a harder metal such as steel and nickel base alloys facilitated the drawing of wires, bars, tubes and other shapes. A number of different processes for applying such coatings had been proposed, including various hot dip methods. In the hot dip methods a bath of molten lead or other soft metal was ordinarily covered in whole or in part with a molten flux through which the article to be coated was passed into the molten metal bath. While the functions of the flux were not completely understood, it was believed that the flux functioned as a wetting agent and protected the surface of the molten metal bath from oxidation. In carrying out such hot dip operations it was found necessary, in commercial practice, to have a perfectly clean metallic surface on the articles being coated in order to get satisfactory results. Depending upon the metal being coated, such a clean metallic surface was obtained by grinding, pickling, gas reduction etc. Despite care in pickling or otherwise cleaning the surface, drawing difficulties frequently occurred, particularly on the inside surfaces of tubes. The most common drawing difficulty appeared as scoring marks on the surface of the drawn article and in some cases there would be actual metal pick-up on the mandrel or die. Attempts to overcome these difficulties, which appeared to be traceable to uncontrollable pickling and leading practice, were unsuccessful.

I have invented a new flux and process for coating metals and alloys which not only overcomes the difficulties of prior art practice but also makes it possible, when desired, to omit the pickling or cleaning steps and still get satisfactory lead coatings and satisfactory drawing characteristics.

It is an object of the present invention to provide a process of producing a lead coating on metals and alloys which adheres firmly to the underlying foundation.

The present invention embraces superficially oxidized metallic shapes having an adherent lead coating and a process of coating metallic shapes with lead which can be carried out without a preliminary pickling or cleaning operation so that superficially oxidized shapes, e. g., hot rolled articles, may be coated directly with an adherent lead coating.

Further objects of the present invention include a flux and a process for lead coating metals and alloys which will insure a coating of lead having good covering power and firm adherence to the foundation.

5 The present invention also contemplates coating metals and alloys as a step preparatory to a drawing operation, which coating will be of such character as to prevent metal pick-up on the dies and mandrels employed in the drawing operation.

Other objects and advantages of the present invention will become apparent from the following detailed description of the invention taken in conjunction with the drawings in which:

10 Fig. 1 is a ternary chart showing the composition of the flux embodying the present invention;

Fig. 2 depicts schematically the structure of a short metal object that has been coated with lead by the process of the present invention without removing the oxide layer;

15 Figs. 3 and 4 reproduce, respectively, a photograph of a section of a two inch alloy tube after being coated with lead by the method of the present invention and a section of 1 $\frac{1}{8}$  inch tube of a different alloy after being so coated and subsequently drawn to effect about 46% reduction in area in two passes, a portion of the lead coating in each case having been dissolved off with dilute nitric acid to reveal the underlying oxide layer and a part of the oxide layer having been pickled off to show the foundation or base metal; and

20 Fig. 5 is a schematic reproduction of a photomicrograph of a cross section of a tube coated with lead by the process of the present invention taken adjacent to the surface thereof and showing the lead coating adhering to an oxide coating which in turn strongly adheres to the foundation or base metal.

25 30 35 40 45 50 Generally speaking, the present invention contemplates the production of an adherent coating of lead on harder metals and alloys by a hot dip method involving the use of a novel flux composition on a bath of molten lead. The novel flux is composed largely of zinc chloride and ferric chloride and preferably also contains minor amounts of ammonium chloride. Referring to Fig. 1, the field enclosed within the lines A B C D E A represents the operable flux compositions which fall within the ranges:

|                    | Per cent |
|--------------------|----------|
| ZnCl <sub>2</sub>  | 20 to 95 |
| FeCl <sub>3</sub>  | 5 to 55  |
| NH <sub>4</sub> Cl | 0 to 40  |

Preferably the flux composition lies within the field bounded by lines F G H I F corresponding to the ranges:

|                    | Per cent |
|--------------------|----------|
| ZnCl <sub>2</sub>  | 35 to 90 |
| FeCl <sub>3</sub>  | 5 to 35  |
| NH <sub>4</sub> Cl | 5 to 30  |

Other metal halides may also be present without interfering with the operation of the new flux. For example, a flux containing about 67% zinc chloride, 17% sodium chloride, and 16% ferric chloride was found to work satisfactorily. A typical example of a flux that has given excellent results in commercial scale operations contained about 70% zinc chloride, 25% ferric chloride (FeCl<sub>3</sub>.6H<sub>2</sub>O), and 5% ammonium chloride.

The ferric chloride content of the flux, while it may be as high as about 55%, preferably should not exceed about 35%. Above 35% FeCl<sub>3</sub> the flux gives off brown fumes that become especially pronounced at about 55%. If FeCl<sub>3</sub> is increased above 55%, there results an increased viscosity and excessive volatilization of FeCl<sub>3</sub>. It is difficult to obtain consistent leading results when more than about 35% FeCl<sub>3</sub> is used, the flux usually becoming stiff, mushy and pasty which is not conducive to good leading. The minimum amount of ferric chloride which may be satisfactorily used in the process contemplated by the present invention is critical and depends somewhat upon the temperature of the flux, less ferric chloride being required as the temperature increases. Thus, when the temperature of the flux bath is within the range of about 670 to 700° F., at least about 8% ferric chloride is necessary, whereas good results can be had with about 5% ferric chloride when the temperature of the bath is within the range of about 825 to 850° F.

Ammonium chloride preferably is used to the extent of at least about 5%, although satisfactory results have been obtained when the flux

within the temperature range of about 630° F. (10° above the melting point of lead) to 950° F., preferably within the range of about 640° to 700° F., and is covered with a layer of the new flux which is molten at this temperature. The flux preferably is prepared by mixing the ingredients as a thick paste with water before it is poured on the molten lead bath, although a mixture of dry ingredients can be used. A more intimate mixture is obtained in the paste which is easier to melt down. The flux becomes heated by conduction from the molten metal bath and as the temperature of the flux rises above the boiling point of water, the water used in preparing the flux paste evaporates and the flux becomes molten on further heating. After the flux has reached the temperature of the metal bath, the articles to be coated are passed through the molten flux into the molten metal. Tubular articles must be introduced in such a manner that the flux flows through the interior and wets all parts of the inner surface. When this is done a satisfactory adherent lead coating of good covering power is obtained regardless of the condition of the surface of the articles, i. e., whether the hot rolled finish has been removed by pickling or not. This is a new result of great commercial importance since it makes it possible to produce drawn products without the necessity of pickling or otherwise cleaning the metal blanks prior to the drawing operation.

For the purpose of acquainting those skilled in the art with the benefits and advantages of the present invention, the results obtained in leading 7/32 inch hot rolled rounds of a nickel-chromium-iron alloy under various fluxes are given in Table 1. This alloy which is sold under the trade mark "Inconel" contains about 79% nickel, about 13% chromium and the balance iron and minor constituents and impurities. In the hot rolled condition, this alloy is covered with a superficial dark brown to black oxide layer.

Table I

| Ex-<br>ample<br>No. | Cleaning treat-<br>ment | Flux composition (weight percent) |                   |                    |                     | Leading       |                | Coating       |
|---------------------|-------------------------|-----------------------------------|-------------------|--------------------|---------------------|---------------|----------------|---------------|
|                     |                         | ZnCl <sub>2</sub>                 | FeCl <sub>3</sub> | NH <sub>4</sub> Cl | Others              | Temp.,<br>°F. | Time<br>(min.) |               |
| 1                   | Pickled                 | 71                                |                   | 5.5                | 23.5 NaCl           | 700           | 5              | Satisfactory. |
| 2                   | None                    | 71                                |                   | 5.5                | 23.5 NaCl           | 700           | 5              | No coating.   |
| 3                   | do                      | 60                                | 16                | 4                  | 20 NaCl             | 670-700       | 5-8            | Satisfactory. |
| 4                   | Pickled                 | 80                                |                   |                    | 20 NaCl             | 700           | 5              | Do.           |
| 5                   | None                    | 80                                |                   |                    | 20 NaCl             | 700           | 5              | No coating.   |
| 6                   | do                      | 67                                | 16                | 5.5                | 17 NaCl             | 670-700       | 5-8            | Satisfactory. |
| 7                   | Pickled                 | 79.5                              | 15                | 5.5                |                     | 670-700       | 5              | Do.           |
| 8                   | None                    | 79.5                              | 15                | 5.5                |                     | 680-700       | 5              | Do.           |
| 9                   | Pickled                 | 55                                | 15                | 30                 |                     | 670-700       | 10             | Do.           |
| 10                  | None                    | 55                                | 15                | 30                 |                     | 670-700       | 10-15          | Do.           |
| 11                  | Pickled                 | 61.5                              | 8.5               | 15                 | 15 NaCl             | 700           | 5              | Do.           |
| 12                  | None                    | 61.5                              | 8.5               | 15                 | 15 NaCl             | 810-840       | 10-15          | Do.           |
| 13                  | Pickled                 | 73.5                              | 15                |                    | 11.5 CuCl           | 670-700       | 5              | Do.           |
| 14                  | None                    | 73.5                              | 15                |                    | 11.5 CuCl           | 670-700       | 5              | Do.           |
| 14a                 | do                      | 72.8                              |                   |                    | 18.2 NaCl, 9.0 CuCl | 700           | 5              | Very poor.    |

was free from this salt. The effect of ammonium chloride is to facilitate a clean separation of flux from the leaded article when it is removed from the bath and to maintain the fluidity of the flux bath. As ammonium chloride is increased above about 20%, there is a slight increase in the fuming tendency of the bath and above about 40% there is excessive fuming of NH<sub>4</sub>Cl, the flux becomes crusty and cakes at the surface of the lead bath.

In coating wires, bars, tubes and other shapes by the process of the present invention, a molten bath of soft metal such as lead is heated

65 of the foregoing, the flux used for Examples Nos. 7 and 8 had the best combination of properties and it has given very satisfactory results in leading operations on a commercial scale. The rounds of Examples Nos. 9 and 10 were very well covered with lead but the flux fumed considerably at the temperature employed. The flux

70 used in Example No. 12 required a higher temperature to coat unpickled materials than the flux of Example No. 6, for example. The flux of Examples Nos. 13 and 14 was much more viscous than the other fluxes and is less desirable inasmuch as the higher viscosity made it difficult

to obtain perfect coatings on the insides of tubes although good coatings on the outer surface of tubes and rods were obtained. The examples in Table I clearly show that the ferric chloride is the active ingredient which makes it possible to coat uncleared metallic surfaces and that in addition to zinc chloride and ammonium chloride other metallic halides may be present in the flux without impairing its activity.

In Table II are summarized the results obtained in coating Inconel rods and tubes. These blanks had oxide coatings of various characteristics, depending upon the prior treatment. Thus, rods and tubes in the hot rolled condition or which had been subjected to an oxidizing anneal were covered with an oxide coating having a brown to black cast. On the other hand, articles which had been subjected to a reducing anneal following hot rolling were covered with an oxide coating having a greenish hue. The rod of Example No. 15 had a  $\frac{3}{8}$  inch diameter and the flux employed contained about 20%  $\text{FeCl}_3$ , 75%  $\text{ZnCl}_2$  and 5%  $\text{NH}_4\text{Cl}$ . The tubes of Examples 16, 17 and 18 were 8 gauge, 2 inches in diameter and  $4\frac{1}{2}$  feet long and they were coated using a flux of the same composition as Examples 7 and 8.

Table II

| Example No. | Shape | Oxide coating | Cleaning treatment | Leading    |             | Coating                                                        |
|-------------|-------|---------------|--------------------|------------|-------------|----------------------------------------------------------------|
|             |       |               |                    | Temp., °F. | Time (min.) |                                                                |
| 15.         | Rod   | Green         | None               | 670-700    | 5-8         | Satisfactory.                                                  |
| 16.         | Tube  | do            | Pickled            | 680-700    | 5           | Satisfactory on both surfaces.                                 |
| 17.         | do    | do            | None               | 680-700    | 10          | Satisfactory outside, inside not entirely coated in this time. |
| 18.         | do    | Black         | do                 | 700        | 10          | Satisfactory on both surfaces.                                 |

It is more difficult to get a satisfactory adher- 40 ent lead coating of good covering power on articles covered with a green oxide coating than on those having the black to brown oxide coating. The reaction between the flux and the green oxide coating is much more sluggish than the reaction with the brown to black oxide. Satisfactory results in coating Inconel articles covered with the green oxide coating ordinarily can be obtained by allowing a longer time for the reaction to take place or by raising the tempera- 45 ture of the bath or both.

Table III summarizes the results obtained in coating rods of an age hardenable nickel-copper-aluminum alloy sold under the trade mark "K-Monel." These rods were given no cleaning treatment following hot rolling and the surfaces therefore were covered with a layer of oxide having a blue-black to black cast.

Table III

| Ex-<br>ample<br>No. | Flux            |                 |                        | Leading    |             | Coating    |
|---------------------|-----------------|-----------------|------------------------|------------|-------------|------------|
|                     | $\text{ZnCl}_2$ | $\text{FeCl}_3$ | $\text{NH}_4\text{Cl}$ | Temp., °F. | Time (min.) |            |
| 19                  | 87              | 8               | 5                      | 670-700    | 5-8         | Very good. |
| 20                  | 78              | 16              | 5                      | 670-700    | 5-8         | Do.        |
| 21                  | 70              | 25              | 5                      | 670-700    | 5-8         | Do.        |

Articles coated with lead by the process embodying the present invention lend themselves readily to drawing operations.

The lead coated tube of Example No. 16, for example, was given a first draw resulting in a reduction in area of about 32%. The tube had ex-

cellent drawing characteristics and the mandrel showed no signs of injury. The tube was given a second draw resulting in a further reduction in area of 30.5% without an intermediate anneal and without further lead coating. Again the tube had excellent drawing characteristics and the mandrel showed no sign of damage. After a total reduction in area of about 45.6%, close inspection of the inside and outside of the tube showed that the surface was unscratched and completely satisfactory.

The tube of Example No. 17 was drawn in the same manner as Tube No. 16. The outside surface was completely satisfactory but there were some scoring marks on the inside of the tube due to the fact that the reaction time had not been quite sufficient completely to coat the inner surface of the tube. By employing a somewhat higher temperature, a longer time, or both, this difficulty can largely be overcome.

The tube of Example No. 18 was also drawn in the same manner as Examples No. 16 and 17 and it also had excellent drawing characteristics and both the inside and outside surfaces of the drawn tube were excellent.

An Inconel wire covered with a black oxide layer was coated with lead in the same manner as

Example No. 8. It was then given a reduction in area of about 52.3% in 2 passes through a wire drawing die. The wire had excellent drawing characteristics. Thereafter it was subjected to a second draw resulting in about 98.7% reduction in area in 6 passes, without intermediate anneal and without recoating with lead. Minute inspection after the second draw showed that the surface was very smooth and uniform and the results were highly satisfactory.

The new flux has given remarkable improvement in the drawing characteristics of certain iron-nickel-chromium alloys of the Elinvar type which require heavy cold reduction in order to produce substantially constant modulus of elasticity. In prior art practice in which a flux corresponding substantially to that used in Example No. 1 was used, it was necessary to carry out the drawing in 2 steps of three passes, each separated by an intermediate anneal followed by reloading. When the new flux was used, the material was drawn to finished size with 93.5% reduction in area in 7 passes without intermediate anneal and without reloading.

The leading coating process of the present invention, as will be clear from the foregoing specific examples, can be carried out on metal articles that have been cleaned by pickling or otherwise to remove the oxide or other surface layer, but its greatest advantage resides in the ability of the new flux to coat articles without the necessity for removing the oxide or other surface layer. This is a new result that the prior art was not able to achieve and it produces a new article of manufacture, namely a composite article of manufacture having a foundation or base

metal layer, an adherent oxide layer and an adherent lead coating. The structure of this new article of manufacture is depicted schematically in Fig. 2, in which the thicknesses of the lead coating and the oxide layer have been exaggerated for purposes of illustration. Fig. 3 is a reproduction of a photograph taken of a short section of a 2 inch K-Monel tube which had been coated in accordance with the present invention without removal of the oxide surface which was formed during the conventional process of manufacturing the tube. The zone at the left shows the tube in the as leaded condition. The dark middle zone shows the black oxide layer after the lead coating had been removed with dilute nitric acid. The zone at the right shows the foundation or base metal after pickling off the oxide layer. The lead coating was very adherent to the oxide layer which in turn adhered very strongly to the base metal.

Fig. 4 is a reproduction of a photograph of a 1 $\frac{1}{8}$  inch Inconel tube which had been coated without pickling in accordance with the process of the present invention and then drawn to effect 45.6% reduction in area in two passes. The zone at the left shows the lead coating which is still intact after the drawing operation. The dark middle zone shows the black oxide remaining on the surface of the foundation metal after the lead coating had been removed with dilute nitric acid. The zone at the right shows the foundation metal after the oxide layer had been removed by pickling. The drawing characteristics of the tube were excellent despite the presence of the oxide layer under the lead.

While the mechanism of the action of the new flux is not thoroughly understood, it is believed that when articles which have not been cleaned or pickled are introduced into the new flux, a reaction takes place between the flux and the oxide layer. This reaction apparently does not completely remove the oxide coating from the surface of the article because articles which have been satisfactorily coated and drawn and from which the lead has been removed by deleading in dilute nitric acid still have an adherent coating of oxide, as may be seen in Fig. 4. It may be that the oxide layer is penetrated by the flux to provide a plurality of tenacles of lead on the underside of the coating extending into contact with the base metal itself but definite evidence in support of this theory is lacking. Whatever the mechanism of the reaction may be, the results of the reaction based upon a large number of experiments have been found to produce a very definite improvement in the lead coating obtained and in the drawing characteristics of the coated article, as compared with prior art practice, particularly where the material was not cleaned or pickled prior to the leading operation.

Ferric fluoride may be used to replace ferric chloride either in whole or in part in the flux embodying the present invention. Experiments made with  $FeF_3$  indicate that this compound is less reactive than  $FeCl_3$  since a longer leading time is required under comparable conditions to get equivalent results. It also has a higher melting point and is more expensive than ferric chloride. The following are typical examples of satisfactory fluxes in which  $FeF_3$  was used instead of  $FeCl_3$ :

| FeF <sub>3</sub><br>Per cent | ZnCl <sub>2</sub><br>Per cent | NH <sub>4</sub> Cl<br>Per cent |
|------------------------------|-------------------------------|--------------------------------|
| 5                            | 90                            | 5                              |
| 10                           | 85                            | 5                              |
| 20                           | 75                            | 5                              |

10 Although the present invention has been described in connection with certain specific embodiments, it is to be clearly understood that these examples have been given by way of illustration and not by way of limitation. Modifications and variations in the flux composition and leading practice are possible, as those skilled in the art will readily understand, and are contemplated as being within the scope of the present invention, as defined in the appended claims.

I claim:

- 20 1. A lead coating bath characterized by the ability to form an adherent layer of lead on oxide coated nickel and nickel alloys comprising a lead bath and a floating flux blanket containing about 20% to 95% of zinc chloride and about 5% to 35% of iron salt from the group consisting of ferric chloride and ferric fluoride, the recited iron and zinc compounds constituting not less than 60% of the total composition of the flux.

25 2. A flux adapted for preparing metal articles for an adherent lead coating which comprises about 5% to 35% of ferric chloride, about 5% of ammonium chloride, and the balance substantially all zinc chloride.

30 3. A metal halide flux for use as a molten covering in a lead coating bath consisting essentially of from 35% to 90% zinc chloride and from 5% to 35% of an iron halide from the group consisting of ferric chloride and ferric fluoride, the remainder of the composition being made up by at least one halide salt selected from the group consisting of alkali metal and ammonium halides.

35 4. A lead coating flux consisting essentially of zinc chloride, ferric chloride and ammonium chloride, being present in proportions bounded by the curve F G H I F of the drawings.

40 5. A lead coating flux consisting of zinc chloride 79.5%, ferric chloride 15%, and ammonium chloride 5.5%.

45 6. A lead coating flux consisting of zinc chloride 67%, sodium chloride 17%, and ferric chloride 16%.

50 7. A lead coating flux consisting of zinc chloride 70%, ferric chloride 25%, and ammonium chloride 5%.

55 8. The method of lead coating articles made of nickel and nickel alloys without cleaning and removal of the hot rolled oxide surface, comprising pretreating the uncleansed articles in a molten flux bath containing about 8% to 35% of iron salt from the group consisting of ferric chloride and ferric fluoride and 35% to 90% zinc chloride, the recited iron and zinc compounds constituting not less than 60% of the total composition of the flux, said bath being heated to a temperature range of between 670° to 700° F., thereafter immersing the pretreated articles in molten lead, and withdrawing the articles with a firmly adhering coating of lead covering the same.

## EUGENE JOSEPH KALIL.